

# UNITED STATES PATENT OFFICE.

WILHELM MATT, OF NEW YORK, N. Y., ASSIGNOR TO THE PATENT MARBLE VENEER COMPANY, OF SAME PLACE.

## ARTIFICIAL STONE FOR VENEERS, MOLDED ARTICLES, &c.

SPECIFICATION forming part of Letters Patent No. 289,112, dated November 27, 1883.

Application filed May 11, 1883. (No specimens.)

*To all whom it may concern:*

Be it known that I, WILHELM MATT, of the city, county, and State of New York, have invented a new and useful Composition of Matter or Artificial Stone for Veneers, Molded Articles, &c.; and I do hereby declare that the following is a full and exact description of the same.

My invention relates to a new composition 10 of matter for use as a veneer or artificial surface for wood, plaster, papier-maché, ceramics, &c., and the same is an improvement upon the composition described in Letters Patent No. 266,493, granted to me October 24, 1882.

15 The composition composing the subject of my invention is best made in the following manner: Take, say, ten pounds of copper-glue, and soak the same in about eighteen pounds of water, and then completely dissolve

20 the glue by boiling with overheated steam. During the boiling I add to this solution of hot glue about ten pounds of fine asbestos and thoroughly stir and mix the fibers of the same with the mass of glue. In the meantime I

25 take about one-half a pound of boiled linseed-oil varnish and one-half pound of colophony and melt them together, and while in a boiling condition add them slowly to the aforesaid hot solution of glue and asbestos, and I keep

30 the mass in a constant state of agitation by stirring until no more foam or air-bubbles appear. To the hot mass I now add about one pound of glycerine and stir as before, and I then add as a final material, to complete the

35 combination of materials, about one and a half pound of thick Venetian turpentine. If it is desired, the compound may now be stiffened by the addition of French chalk, China clay, or other equivalent material, and the

40 compound may be colored by the addition of such pigments as taste or fancy may dictate. The plastic compound thus produced is made ready for use as a veneer by being rolled out

45 into thin sheets, which are united to the surface to be covered by coating both the sheet of composition and the surface to be veneered each with a film of hot glue, in thin solution, and then pressing the two together, as in the ordinary process of veneering wood. In this 50 manner not only all manner of wood surfaces

may be veneered with the compound; but it may be applied to plaster walls, to papier-maché, and in fact to all surfaces to which the glue will adhere. The composition will harden within twenty-four hours and become as 55 hard as stone, and presents a smooth finished surface, which admits of receiving a very high polish. This polish may be produced by first rubbing down with pumice-stone and oil of turpentine and finishing with sandarac-polish 60 in the usual manner. When applied to a wooden surface, this composition adheres so closely as to become apparently an integral part therewith, and it is so hard that it will not break or peel off, but will in some cases 65 be more durable than the body of the article, the combination of the glue and the glycerine in the compound making it both tough and elastic.

For producing an imitation of marble with 70 this compound, I take suitable colors and mix separately with each a proportion of finely-pulverized steatite or kaolin, each color being placed in a separate heap upon a marble slab. The center of each heap is hollowed out to receive a quantity of the hot fluid solution of glue, asbestos, linseed-oil varnish, colophony, glycerine, and turpentine sufficient to reduce the mass to a pasty condition. When the several colors are thus made ready, each in the 80 form of paste of proper consistency, they are kept ready for use by enfolding them in a damp cloth. When required for use, the separate masses of color are steamed until heated through and through and fully softened, and 85 are placed upon the marble slabs in rolls, which are properly laid together and interfolded, rolled out with a suitable metallic roller, folded, and again rolled into a thin sheet, which will finally become veined in a beautiful 90 imitation of marble.

The proportion of the several ingredients herein named are those best adapted to produce the desired results. They may, however, be slightly varied without departing 95 from my invention.

I claim as my invention—

1. A composition of matter for veneering or molding purposes, produced by an admixture, in substantially the proportions and man- 100

ner described, of a solution of glue with asbestos, linseed-oil varnish, colophony, glycerine, and turpentine, for the purposes herein set forth.

- 5 2. A composition of matter for veneering and marbleizing purposes, produced by an admixture, in substantially the proportions and manner described, of a solution of glue with asbestos, linseed - oil varnish, colophony, 10 glycerine, turpentine, steatite or kaolin, and coloring-pigments, for the purposes herein set forth.
3. The composition herein specified, com-

posed of glue, asbestos, linseed-oil varnish, colophony, glycerine, and turpentine, as set forth.

4. The composition herein specified, composed of glue, asbestos, linseed-oil varnish, colophony, glycerine, turpentine, steatite or kaolin, and coloring-pigments, as set forth. 20

Signed by me this 9th day of May, A. D. 1883.

WILHELM MATT.

Witnesses:

HAROLD SERRELL,  
CHAS. PUTZEL.